

3,230,700

ROCKET PROPULSION METHOD USING HYDROCARBON FUELS CONTAINING AMINOALKYL ACRYLATE POLYMERS  
Olaf E. Larsen, Bartlesville, Okla., assignor to Phillips Petroleum Company, a corporation of Delaware  
No Drawing. Filed Oct. 27, 1958, Ser. No. 769,952  
10 Claims. (Cl. 60—35.4)

This invention relates to rocket propellants. In one aspect, this invention relates to the addition of a small amount of a surface active agent to a liquid hydrocarbon fuel to enhance rocket motor performance characteristics when said fuel is used with a nitric acid oxidizer in a rocket motor.

Rocket motors are operated by burning a mixture of fuel and oxidant in a combustion chamber and causing the resulting gases to be expelled through a nozzle at high velocity. Liquid propellants are frequently preferred over solid propellants where it is necessary to vary thrust during flight. Liquid propellants can be classified as bipropellants and as monopropellants and the latter are either a single compound or mixtures of compounds. The principal elements of a rocket motor utilizing a liquid fuel comprise a combustion chamber, exhaust nozzle, an injection system, and propellant control valves. The propellant gases are produced in the combustion chamber at pressures governed by the chemical characteristics of the propellant, its rate of combustion, and the cross-sectional area of the nozzle throat. The gases are ejected into the atmosphere through the nozzle with supersonic velocity. The function of the nozzle is to convert the pressure of the propellant gases into kinetic energy. The reaction of the discharge of the propellant gases constitutes the thrust developed by the rocket motor.

The present invention relates to utilizing a liquid bipropellant system in a rocket motor. In the operation of rocket motors utilizing this system of propellants, it is usually desirable to inject the oxidizer component and the fuel component into the combustion chamber of the rocket motor as separate streams. If the fuel component is a hypergolic fuel, it is necessary that said fuel component and said oxidizer component be introduced as separate streams so that the initial contact occurs in the combustion chamber because spontaneous ignition occurs upon said initial contact. If, however, the fuel component is a non-hypergolic fuel, the oxidizer component and the fuel component can be mixed immediately prior to introduction into the combustion chamber and the introduced mixture, which is introduced as a single stream, can be ignited by any suitable ignition means, such as an electrical igniter.

A number of problems have been encountered in the development of liquid bipropellant rocket motors using hydrocarbon fuels and nitric acid oxidizers. Rapid and smooth ignition and stable combustion are two major problem areas related to the physical and chemical compositions of the reactants. Most hydrocarbons, and hydrocarbon blends such as the JP-type fuels, are non-hypergolic with nitric acid oxidizers and require an independent source of energy for ignition. Both low frequency and high frequency combustion oscillations in the combustion chamber, such as those referred to as chugging and screaming respectively, and which may result in unstable operation of the rocket motor, or even flame out, are forms of combustion instability that are effected by fuel type.

When a nitric acid oxidizer and a liquid hydrocarbon are mixed, certain precursor reactions take place with the evolution of considerable thermal energy during the initial exothermic reactions which occur upon mixing. It has been found that a correlation exists between the amount of thermal energy released when a liquid hydrocarbon is

mixed with a nitric acid oxidizer and the operation of the rocket motor when said fuel is burned therein. It has been found that the greater the amount of total thermal energy released, the more suitable the fuel is as a fuel for a rocket motor, i.e., more rapid and smooth ignition, and more stable combustion will occur in the combustion chamber of the rocket motor. The amount of thermal energy released upon mixing of a liquid hydrocarbon fuel and a nitric acid oxidizer can be determined by measuring the amount of temperature increase which occurs when said fuel is added to said oxidizer. It has been found that the rate-of-temperature rise is related to the ease of ignition of the fuel and oxidizer mixture and the over-all burning process, and the total amount of energy produced is related to the over-all combustion stability.

In accordance with the invention, it has been found that the reactions between a normally liquid hydrocarbon and a nitric acid oxidizer can be enhanced by incorporating a surface active agent in said normally liquid hydrocarbon. Enhancing the reaction between said liquid hydrocarbon and the nitric acid oxidizer also enhances the performance characteristics of the rocket motor wherein said bipropellant system is used. However, as discussed further herein-after, all surface active agents are not effective to enhance the reaction between liquid hydrocarbons and nitric acid.

Thus, broadly speaking, the present invention resides in the use of a normally liquid hydrocarbon fuel having dissolved therein a copolymer of a predominantly non-polar alkyl acrylate monomer with an aminoalkyl acrylate monomer which contains a basic nitrogen atom, as the fuel component in a nitric acid-liquid hydrocarbon bipropellant system for developing thrust in a reaction motor, said copolymer being present in an amount sufficient to enhance the reaction between liquid hydrocarbons and nitric acid.

An object of this invention is to provide an improved liquid bipropellant system for use in rocket motors. Another object of this invention is to provide an improved method for the operation of rocket motors utilizing a liquid bipropellant system. Still another object of this invention is to enhance the reaction between a normally liquid hydrocarbon fuel and a nitric acid oxidizer in a liquid bipropellant system. Other aspects, objects, and advantages of this invention will be apparent to those skilled in the art in view of this disclosure.

Thus, according to the invention, there is provided a method for developing thrust by the combustion of bipropellant components in a combustion chamber of a reaction motor, which method comprises: injecting a nitric acid oxidizer component containing at least about 70 weight percent  $\text{HNO}_3$  and a normally liquid hydrocarbon fuel component into said combustion chamber; igniting and burning a mixture of said components in said combustion chamber to form products of combustion; and exhausting said products of combustion from said motor; said fuel component comprising from 99 to 95 weight percent of a normally liquid hydrocarbon and from 1 to 5 weight percent of a copolymer formed by copolymerizing, in parts by weight per 100 parts of monomers, from 5 to 50 parts of at least one monomer selected from the group of alkyl acrylate esters having the formula



65 with from 95 to 50 parts of at least one monomer selected from the group consisting of aminoalkyl acrylates having the formula



wherein each  $R_1$  is selected from the group consisting of hydrogen, and alkyl radicals containing from 1 to 3 carbon atoms; each  $R_2$  is an alkyl radical containing from 10 to 18 carbon atoms; each  $R_3$  is an alkylene radical containing from 1 to 8 carbon atoms; and each  $R_4$  is selected from the group consisting of hydrogen, and alkyl radicals containing from 1 to 18 carbon atoms.

Suitable predominantly non-polar alkyl acrylate monomers for use in the practice of the invention include, among others, those given in Table I below:

TABLE I.—ALKYL ACRYLATE MONOMERS

|                         |
|-------------------------|
| Decyl methacrylate      |
| Dodecyl acrylate        |
| Dodecyl methacrylate    |
| Tetradecyl methacrylate |
| Tridecyl methacrylate   |
| Hexadecyl methacrylate  |
| Octadecyl methacrylate  |
| Dodecyl ethacrylate     |
| Hexadecyl ethacrylate   |
| Dodecyl propacrylate    |
| Hexadecyl propacrylate  |

Aminoalkyl acrylate monomers containing a basic nitrogen atom which are suitable for use in the practice of the invention include, among others, those given in Table II below:

TABLE II.—AMINOALKYL ACRYLATES

|                                                 |
|-------------------------------------------------|
| Aminomethyl acrylate                            |
| Aminomethyl methacrylate                        |
| Aminopentyl methacrylate                        |
| Aminopropyl methacrylate                        |
| Aminopentyl acrylate                            |
| Aminohexyl methacrylate                         |
| Aminoheptyl methacrylate                        |
| Aminoctyl methacrylate                          |
| Aminomethyl ethacrylate                         |
| Aminomethyl propacrylate                        |
| Aminohexyl ethacrylate                          |
| Aminoctyl ethacrylate                           |
| Amino-2-ethylhexyl acrylate                     |
| Dimethylaminomethyl methacrylate                |
| Diethylaminoethyl acrylate                      |
| Diisopropylaminoethyl methacrylate              |
| Dihexylaminoethyl methacrylate                  |
| Di-(2,4,6-triethyloctyl)aminoethyl methacrylate |
| Didodecylaminoethyl methacrylate                |
| Dioctadecylaminoethyl methacrylate              |
| Dimethylaminopropyl methacrylate                |
| Dimethylaminobutyl acrylate                     |
| Dimethylaminopentyl methacrylate                |
| Dimethylaminoctyl methacrylate                  |
| Dihexylaminoctyl methacrylate                   |
| Dihexylaminoctyl ethacrylate                    |
| Dioctylaminoctyl methacrylate                   |
| Dimethylamino-(2-ethylpropyl) acrylate          |

The above-mentioned acrylate monomers can be copolymerized by any method known to those skilled in the art to form the copolymers used in the practice of the invention. Normally these copolymers are prepared by emulsion, bulk, and solution polymerization processes. For example, said monomers can be emulsified in water and a polymerization catalyst such as benzoyl peroxide added thereto. The polymerization can be effected at temperature in the range of 20 to 150° C. until the desired degree of polymerization has been effected. The resulting copolymer can be recovered from the reaction mixture after coagulation thereof with sodium chloride. Further information regarding the details of said copolymerization can be found in U.S. Patents 2,138,031 and 2,138,763, issued to George D. Graves on November 29, 1938. Said monomers are preferably copolymerized in amounts, in parts by weight per 100 parts of monomers, ranging from

5 to 50 parts of at least one of said alkyl acrylate monomers with from 95 to 50 parts of at least one of said amino alkyl acrylate monomers.

Suitable copolymers prepared from the above described monomers and which are suitable for use in the practice of the invention include among others the following:

TABLE III

| Monomer Ratio | Copolymers                                                   |
|---------------|--------------------------------------------------------------|
| 10            |                                                              |
| 55/45.....    | Decyl methacrylate/aminopentyl methacrylate.                 |
| 75/25.....    | Dodecyl methacrylate/aminopentyl acrylate.                   |
| 70/30.....    | Tetradecyl methacrylate/aminooctyl methacrylate.             |
| 65/35.....    | Tridecyl methacrylate/aminooctyl ethacrylate.                |
| 95/5.....     | Dodecyl ethacrylate/aminooctylhexyl acrylate.                |
| 15            | Hexadecyl ethacrylate/dioctadecylaminoethyl acrylate.        |
| 90/10.....    | Hexadecyl ethacrylate/decadecylaminoethyl acrylate.          |
| 85/15.....    | Hexadecyl ethacrylate/dioctadecylaminoethyl methacrylate.    |
| 50/50.....    | Dodecyl propacrylate/dimethylaminopropyl methacrylate.       |
| 85/15.....    | Hexadecyl propacrylate/dimethylaminoctyl methacrylate.       |
| 20            | Decyl methacrylate/dihexylaminoctyl methacrylate.            |
| 80/20.....    | Dodecyl methacrylate/dimethylamino-(2-ethylpropyl) acrylate. |
| 95/5.....     | Hexadecyl methacrylate/aminooctyl methacrylate.              |
| 90/10.....    | Octadecyl methacrylate/didodecyl aminoethyl ethacrylate.     |
| 50/60.....    | Dodecyl methacrylate/diethylaminoethyl methacrylate.         |
| 95/5.....     | Decyl methacrylate/diethylaminoethyl methacrylate.           |
| 25            | Dodecyl methacrylate/diethylaminoethyl methacrylate.         |
| 90/10.....    | Decyl methacrylate/diethylaminoethyl methacrylate.           |
| 80/20.....    | Dodecyl methacrylate/diethylaminoethyl methacrylate.         |

30 When the surface active agents of the invention are used to enhance the reaction between the normally liquid hydrocarbon and the nitric acid oxidizer, said surface active agents are dissolved in said hydrocarbon in an amount preferably within the range of 1 to 5 weight percent, based on said hydrocarbons. However, in some instances larger and smaller amounts can be effectively used.

In the bipropellants used in the practice of the invention, the ratio of the liquid hydrocarbon fuel component to the nitric acid oxidizer component is preferably near stoichiometric. Said ratio can be in the range of 0.75 to 40 1.25 times that of the stoichiometric amount. The stoichiometric amount of oxidizer is defined as the amount required to obtain complete combustion to nitrogen, carbon dioxide, and water. In computing said stoichiometric amount of oxidizer, consideration is given to the amount of surface active agent which is dissolved in the normally liquid hydrocarbon. Thus, the stoichiometric amount of oxidizer includes the amount necessary to oxidize said surface active agents as well as the amount necessary to oxidize the normally liquid hydrocarbon with which the nitric acid is mixed in the combustion chamber of the reaction motor. A slightly fuel-rich mixture is usually required to give an optimum rocket motor performance.

55 Since water tends to retard combustion of the acid with the liquid hydrocarbon fuel, the nitric acid used in a propellant system is preferably substantially free of water. Thus, the presently most preferred oxidizer is anhydrous nitric acid. However, other more dilute nitric acids can be used in the practice of the invention. White fuming nitric acids and red fuming nitric acids of varying concentrations are available commercially, and all are useful in the practice of this invention. White fuming nitric acid usually contains about 90 to 99 weight percent  $HNO_3$ , from 0 to 2 weight percent  $NO_2$ , and up to about 10 weight percent water. Red fuming nitric acid usually contains about 70 to 90 weight percent  $HNO_3$ , from 2 to 25 weight percent  $NO_2$ , and up to about 10 weight percent water. Of course, mixtures of the above-described acids can be employed to give an acid having any intermediate composition, and all are useful as oxidizers in the practice of this invention. Thus, it has been found that nitric acids of all types containing at least about 70 weight percent  $HNO_3$  are useful as oxidizers in the practice of this invention.

70 The following examples will serve to further illustrate the invention:



3. The method of claim 1 wherein said copolymer is 90:10 dodecyl acrylate/aminoethyl acrylate.
4. The method of claim 1 wherein said copolymer is 50:50 hexadecyl methacrylate/aminoethyl methacrylate.
5. The method of claim 1 wherein said copolymer is 95:5 octadecyl ethacrylate/didodecyl aminoethyl ethacrylate.
6. The method of claim 1 wherein said copolymer is 90:10 dodecyl methacrylate/diethylaminoethyl methacrylate.
7. The method of claim 1 wherein said copolymer is 80:20 dodecyl methacrylate/diethylaminoethyl methacrylate.
8. The method of claim 1 wherein said copolymer is 55:45 decyl methacrylate/aminopentyl methacrylate.
9. The method of claim 1 wherein said copolymer is 75:25 dodecyl methacrylate/aminopentyl acrylate.

10. The method of claim 1 wherein said copolymer is 95:5 dedecyl ethacrylate/amino-2-ethylhexyl acrylate.

## References Cited by the Examiner

| UNITED STATES PATENTS |           |         |                             |
|-----------------------|-----------|---------|-----------------------------|
| 5                     | 2,461,797 | 2/1949  | Zwicki _____ 60-35.4        |
|                       | 2,573,471 | 10/1951 | Malina et al. _____ 60-35.4 |
|                       | 2,604,453 | 7/1952  | Popkin _____ 44-62          |
|                       | 2,697,656 | 12/1954 | Stayner.                    |
| 10                    | 2,697,657 | 12/1954 | Stayner.                    |

## FOREIGN PATENTS

734,632 8/1955 Great Britain.

15 CARL D. QUARFORTH, *Primary Examiner.*  
LEON D. ROSDOL, *Examiner.*

**UNITED STATES PATENT OFFICE**  
**CERTIFICATE OF CORRECTION**

Patent No. 3,230,700

January 25, 1966

Olaf E. Larsen

It is hereby certified that error appears in the above numbered patent requiring correction and that the said Letters Patent should read as corrected below.

Column 6, line 37, for "combusion" read -- combustion --; column 7, line 6, for "95.5" read -- 95:5 --; column 8, line 2, for "dedecyl" read -- dodecyl --.

Signed and sealed this 28th day of June 1966.

(SEAL)

Attest:

ERNEST W. SWIDER

Attesting Officer

EDWARD J. BRENNER

Commissioner of Patents

UNITED STATES PATENT OFFICE  
CERTIFICATE OF CORRECTION

Patent No. 3,230,700

January 25, 1966

Olaf E. Larsen

It is hereby certified that error appears in the above numbered patent requiring correction and that the said Letters Patent should read as corrected below.

Column 6, line 37, for "combusion" read -- combustion --; column 7, line 6, for "95.5" read -- 95:5 --; column 8, line 2, for "dedecyl" read -- dodecyl --.

Signed and sealed this 28th day of June 1966.

(SEAL)

Attest:

ERNEST W. SWIDER

Attesting Officer

EDWARD J. BRENNER

Commissioner of Patents